

[54] MINIMIZING CRAZING OF HOT-DIP ALUMINUM COATINGS

3,639,107 2/1972 Thompson ..... 117/114 C

[75] Inventor: **Ralph W. Leonard**, Plum Borough, Pa.[73] Assignee: **United States Steel Corporation**, Pittsburgh, Pa.[22] Filed: **Sept. 20, 1972**[21] Appl. No.: **290,612**[52] U.S. Cl. .... **117/50**, 117/114 C[51] Int. Cl. .... **C23c 1/08**

[58] Field of Search..... 117/51, 114 C, 50, 114 R

## [56] References Cited

## UNITED STATES PATENTS

2,731,362 1/1956 Brondyke..... 117/51

## OTHER PUBLICATIONS

Handbook of Chemistry and Physics, Chemical Rubber Publishing Co., 1949, pages 1975-1976.

*Primary Examiner*—Ralph S. Kendall*Assistant Examiner*—Jacqueline Ware*Attorney, Agent, or Firm*—Arthur J. Greif

[57]

## ABSTRACT

The crazing resistance of hot dip Al coatings is substantially improved by adding from about 0.2 to 1.5 percent Mn to the molten Al bath.

5 Claims, 1 Drawing Figure



PATENTED OCT 15 1974

3,841,894



## MINIMIZING CRAZING OF HOT-DIP ALUMINUM COATINGS

This invention relates to a hot-dipped, aluminized ferrous product with decreased tendency to crazing and to a method for producing same.

The art commonly employs two basically different molten baths for hot-dip aluminizing of ferrous substrates (sheet, strip, wire). For the production of bright coated articles, the Si content is kept to minimum or residual values, generally below 0.25%. However, this type of coated article is not easily formed, due to the formation of a brittle iron-aluminum alloy layer at the interface between the coating and ferrous substrate. When formable, adherent coatings are required, the art generally employs from about 4 to 11% Si in the bath to retard the rate of alloying between the bath metal and the ferrous substrate. The bulk of this Si is generally present as a discrete phase in the coating. Although significantly more adherent, these latter coatings nevertheless tend to craze, i.e., form fine cracks on the tension side of a formed article. During subsequent exposure, a detrimental iron-rust stain quickly develops in the vicinity of these cracks.

It is therefore an object of this invention to provide a method for minimizing the crazing tendency of hot-dip Al-Si coatings.

Other objects and advantages of the invention will be more apparent from a reading of the following description taken in conjunction with the appended claims, and the drawings, in which:

The FIGURE is an illustration of a bend-test specimen for the evaluation of crazing tendency.

Initial studies on the causes of crazing revealed that the cracks propagated through massive needle-shaped particles in the coating. Electron-probe microanalysis of these particles revealed that they contained iron, aluminum and silicon in combination. (Iron is always present in aluminum-coating baths. It accumulates to an equilibrium concentration, up to about three percent, by dissolution from the rigging and incoming strip.) It is believed that these particles are the brittle, intermetallic compound  $Fe_2Si_2Al_9$ . The crystal structure of this compound is triclinic, and because of the unsymmetrical nature of this lattice type, it grows as platelets when it is the primary phase to solidify. These characteristics of  $Fe_2Si_2Al_9$  explain why the particles exhibit cleavage fracture during forming or bending op-

erations. It would therefore appear that the crack propagation tendency of these particles could be diminished if their morphology could be altered. It has now been found that the addition of from about 0.2 to about 1.5 weight % Mn to the aluminum-silicon bath will produce a more desirable globular-shaped primary constituent (wherein Fe, Al, Si and Mn are in combination) in the final coating. The beneficial effect of such Mn additions is evidenced in the following examples.

Sheet samples (26 gage) were coated in aluminum-silicon alloy bath compositions containing a variety of Mn and Fe concentrations. (See Table I) Prior to coating, the samples were cleaned in trichlorethylene, pickled for four minutes in ten percent HCl solution, and fluxed by immersion in a saturated aqueous solution of  $K_2ZrF_6$ . After fluxing, the samples were dried so as to leave a residue of powdered flux. The samples employed in the bend tests were coated using identical conditions, i.e., a bath temperature of 1300°F and an immersion time of 60 seconds. Excess coating metal and oxide residue were removed from the coated sheets by use of an air-knife. Crazing resistance was determined in controlled bend tests as described in ASTM Spec. A525-71. Severity of crazing was evaluated by examination of the tension side at 30x magnification, wherein severity was rated as follows: 0—no crazing, 1—light crazing, 2—medium crazing and 3—heavy crazing. After a flat bend (0T), each sample was bent again so that the next bend was over one sheet thickness (1T). Samples were then bent over increasing sheet thicknesses (see the FIGURE) until the number of sheet thicknesses was reached in which no crazing was observed. Results are reported in Table I for both (a) the number of sheet thicknesses over which samples were bent to obtain no crazing, and for (b) the 3T bend condition. For each composition, the ratings reported are the average of from four to eight different samples.

The beneficial effect provided by the purposeful addition of Mn (baths D through O) can readily be seen from the above results. Thus, while additions within the range of from about 0.2 to 0.80% Mn provided the maximum resistance, even higher amounts of Mn provided some enhancement in crazing resistance over the baths containing essentially no Mn (baths A through C).

TABLE I

| Coating-Bath Designation | Comparison of Crazing Tendency          |      |      | Number of Sheet Thicknesses to Obtain No Crazing | Rating for 3T Bend |     |
|--------------------------|-----------------------------------------|------|------|--------------------------------------------------|--------------------|-----|
|                          | Bath <sup>(1)</sup> Composition - Wt. % | Mn   | Fe   | Si                                               |                    |     |
| A                        |                                         | 0.03 | 2.2  | 6.9                                              | 7.3                | 1.4 |
| B                        |                                         | 0.01 | 2.5  | 6.6                                              | 8.8                | 2.3 |
| C                        |                                         | 0.01 | 2.67 | 7.3                                              | 7.3                | 1.5 |
| D                        |                                         | 0.23 | 2.5  | 7.6                                              | 3.4                | 0.4 |
| E                        |                                         | 0.37 | 2.5  | 7.4                                              | 3.5                | 0.5 |
| F                        |                                         | 0.54 | 0.90 | 7.7                                              | 2.2                | 0   |
| G                        |                                         | 0.52 | 1.71 | 7.6                                              | 3.8                | 0.4 |
| H                        |                                         | 0.48 | 2.37 | 7.6                                              | 4.1                | 0.8 |
| I                        |                                         | 0.63 | 1.22 | 7.7                                              | 3.0                | 0.4 |
| J                        |                                         | 0.73 | 0.82 | 7.9                                              | 3.0                | 0   |
| K                        |                                         | 0.73 | 1.47 | 7.8                                              | 2.8                | 0.2 |
| L                        |                                         | 0.76 | 2.31 | 7.8                                              | 4.0                | 0.5 |
| M                        |                                         | 0.87 | 1.26 | 7.5                                              | 5.7                | 1.6 |
| N                        |                                         | 0.99 | 1.04 | 8.0                                              | 5.6                | 1.5 |
| O                        |                                         | 1.41 | 0.93 | 7.8                                              | 5.4                | 1.0 |

<sup>(1)</sup> Balance Aluminum

The benefits of this invention may therefore be achieved by utilizing the following procedure. The cleaned strip is bright annealed under a controlled atmosphere, thereby obviating the need for fluxing. The annealed strip is cooled, preferably entering the coating bath at a temperature slightly above that of the bath. To prevent oxidation, the strip is maintained in a controlled atmosphere between the annealing furnace and the coating bath, thus permitting the strip surface to alloy readily with the molten bath metal and form a continuous protective coating. The coated strip is then passed through an appropriate device, e.g. an air knife, for final control of the coating weight. Typical coating weights or thicknesses for sheet product vary from about 0.20 to about 1.0 ounces per square foot of sheet (i.e., about 0.4 to 2.0 mils thick per side).

The coating bath generally contains from about 7 to about 9 percent silicon and is maintained at temperatures ranging from about 1,180°F to about 1,300°F. A preferred practice employs a Mn content of about 0.4 to 0.8 percent, in a bath maintained at a temperature of 1,200°-1,250°F, wherein iron content thereof will be less than about 1.5 percent. It has been found that manganese contents within the above preferred range reduces the maximum iron solubility from about 2.5 percent (manganese-free bath) to less than about 1.5 percent. Thus, the addition of manganese offers a further

advantage in that the reduced iron solubility decreases the rate of attack on the rigging.

I claim:

1. In the method for hot-dip aluminizing of ferrous substrates to produce a protective coating thereon, which comprises; cleaning said substrate and thereafter passing said substrate through a bath of molten aluminum consisting essentially of from about 4 to 11% Si, from about 0.1 to about 3.0% Fe,
- 10 the improvement which comprises, adding Mn to said molten bath in an amount sufficient to maintain a concentration of from about 0.2 to about 1.5 percent.
- 15 2. The method of claim 1, wherein the bath is maintained at a temperature of from about 1,180°F to 1,300°F and the Mn content of the bath is within the range of from about 0.4 to 0.8 percent.
- 20 3. The method of claim 2, wherein said bath temperature is about 1,200°F to 1,250°F and the Fe content is less than about 1.5 percent.
- 25 4. The method of claim 2, wherein the Si content of said bath ranges from about 7 to about 9 percent.
5. The method of claim 4, wherein the final thickness of said protective coating ranges from about 0.4 to about 2.0 mils; said bath is maintained at a temperature of about 1,200°F to 1,250°F and the Fe content is less than about 1.5 percent.

\* \* \* \* \*

30

35

40

45

50

55

60

65